

# United States Patent Office

3,706,668  
Patented Dec. 19, 1972

1

3,706,668  
**POLYPHENYL ETHER LUBRICATING COMPOSITIONS**

Frank S. Clark, 4561 McPherson Ave.,  
St. Louis, Mo. 63108

No Drawing. Filed May 28, 1971, Ser. No. 148,124  
Int. Cl. C10m 1/44

U.S. CL. 252—49.9

10 Claims

**ABSTRACT OF THE DISCLOSURE**

Composition comprising polyphenyl ethers or mixtures thereof and phenoxyphenylphosphinic acids exhibit improved lubricating properties over wide temperature ranges.

This invention relates to improved lubricating compositions comprising polyphenyl ethers and mixtures thereof containing from 3 to 8 aromatic groups and a phenoxyphenylphosphinic acid as a lubricating additive.

Polyphenyl ethers have found wide application as functional fluids in view of their excellent thermal stability and lubricity. For example they have been found to be valuable as hydraulic fluids and as lubricants in motor operation, particularly in jet engines.

Development of synthetic base stocks such as the polyphenyl ether has provided lubricant fluids which are useful at elevated temperature such as 400° to 500° F. It is known that one of the aspects in which the polyphenyl ether base stocks are considered deficient is in their lubricating characteristics. These lubricating characteristics include the load-carrying abilities and wear properties, especially under conditions of high pressures and temperatures reached in the advance design aircraft engines. Thus there is a demand for polyphenyl ethers having improved lubricity properties.

An object of the present invention is to provide base stock compositions employing polyphenyl ethers or mixtures thereof that exhibit improved lubricating properties.

These and other objects will become evident upon consideration of the following specification and example.

It has now been found that compositions comprising a major amount of a polyphenyl ether base stock and a lubricating additive amount of a phenoxyphenylphosphinic acid, have unusual ability to lubricate under high loads at high temperatures.

Any of the well known polyphenyl ether base stocks can be used in accordance with this invention. However, the polyphenyl ether base stocks represented by a member selected from the following formulae are preferred.

(I)



where  $m$  is 2, 3, or 4 such as

bis(m-phenoxyphenyl)ether,  
m-phenoxyphenyl p-phenoxyphenyl ether,  
m-bis(m-phenoxyphenyl)benzene,  
m-[ (m-phenoxyphenyl) (p-phenoxyphenyl) ]benzene,  
p-[ p-phenoxyphenyl ) (m-phenoxyphenyl) ]benzene,  
p-bis(m-phenoxyphenyl)benzene,  
m-bis(p-phenoxyphenyl)benzene and  
o-bis(m-phenoxyphenyl)benzene,

(II)



such as 3,3'-bisphenoxy biphenyl,

2



5 (III)



10

15 such as 1,3,4-triphenoxybenzene,



20

25 (IV) and mixtures thereof.

20 Mixtures of polyphenyl ethers in which the nonterminal phenylene rings are linked through oxygen atoms in the meta and/or para positions, have been found to be particularly suitable. An example of such polyphenyl ether compositions are those containing, in percent by weight, from about 0 to 6% of o-bis(m-phenoxyphenoxy)benzene (1), about 40 to 85% of m-bis(m-phenoxyphenoxy)benzene (2), about 0 to 40% of m-[ (m-phenoxyphenyl) (p-phenoxyphenyl) ]benzene (3), about 0 to 12% of p-bis(m-phenoxyphenyl)benzene (4) about 0 to 10% of p-[ p-phenoxyphenyl ) (m-phenoxyphenyl) ]benzene (5), and about 0 to 6% of m-bis(p-phenoxyphenyl)benzene (6). Typical compositions of such mixtures are listed below. The number of parentheses refers to the compound mentioned above having the same number thereafter.

40

| Component: | Mixtures, percent by weight of components |    |    |      |
|------------|-------------------------------------------|----|----|------|
|            | A                                         | B  | C  | D    |
| (1)-----   | 0                                         | 6  | 5  | 4.5  |
| (2)-----   | 63                                        | 82 | 80 | 43.5 |
| (3)-----   | 31                                        | 0  | 4  | 40   |
| (4)-----   | 0                                         | 12 | 11 | 4    |
| (5)-----   | 0                                         | 0  | 0  | 8    |
| (6)-----   | 6                                         | 0  | 0  | 0    |

50

The amount of the phenoxyphenylphosphinic acid employed in the compositions of this invention can range from about 0.01 to about 0.5% by weight. It is preferred to employ the acids in the compositions of this invention in amounts of from about 0.05 to 0.2% by weight based upon the total composition.

The phenoxyphenylphosphinic acids which can be employed in the compositions of this invention are represented by the formula

60



65

wherein R and R<sup>1</sup> are alkyl of not more than 4 carbon atoms, haloalkyl of not more than 4 carbon atoms and 3 halogen (Cl, Br and F) atoms, halogen (Cl, Br and F) hydroxyl or phenyl, and  $n$  and  $a$  are integers from 0 to 3.

70

Representative groups for R and R<sup>1</sup> in the above formulae include alkyl such as methyl, ethyl, propyl, isopropyl, n-butyl, sec-butyl and t-butyl and haloalkyl such

as chloromethyl, bromomethyl, chloroethyl, bromoethyl, trichloromethyl, tribromomethyl, dichloroethyl, chloro-n-propyl, bromo-n-propyl, bromo-n-butyl, bromo-tert-butyl, 1,3,3-trichlorobutyl and 1,3,3-tribromobutyl.

Phenoxyphenylphosphinic acids represented by the above formula include, for example,

p-phenoxyphenylphosphinic acid,  
o-phenoxyphenylphosphinic acid,  
p-(p-methylphenoxy)phenylphosphinic acid,  
o-(p-methylphenoxy)phenylphosphinic acid,  
p-(o-methylphenoxy)phenylphosphinic acid,  
p-(p-ethylphenoxy)phenylphosphinic acid,  
p-(o-ethylphenoxy)phenylphosphinic acid,  
o-(o-ethylphenoxy)phenylphosphinic acid,  
p-(p-butylphenoxy)phenylphosphinic acid,  
p-(p-chlorophenoxy)phenylphosphinic acid,  
o-(m-chlorophenoxy)phenylphosphinic acid,  
p-(p-phenylphenoxy)phenylphosphinic acid,  
o-(p-phenylphenoxy)phenylphosphinic acid,  
p-(o-hydroxyphenoxy)phenylphosphinic acid,  
p-(m-bromophenoxy)phenylphosphinic acid,  
p-(p-hydroxyphenyl)phenylphosphinic acid,  
o-(m-phenylphenoxy)phenylphosphinic acid,  
o-(p-methylphenoxy)-m-methylphenylphosphinic acid,  
o-(p-methylphenoxy)-m-chloromethylphenylphosphinic acid,  
p-(p-methylphenoxy)-m-trifluoromethylphenylphosphinic acid,  
p-(o-butylphenoxy)-o-trifluoromethylphenylphosphinic acid,  
m-(o-phenylphenoxy)-p-methylphenylphosphinic acid,  
m-(o-methylphenoxy)-o-butylphenylphosphinic acid,  
m-(o-chloromethylphenoxy)-o-methylphenylphosphinic acid,  
o-(m-methylphenoxy)-p-trifluoromethylphenylphosphinic acid,  
o-(m-hydroxyphenoxy)-p-hydroxyphenylphosphinic acid,  
o-(m-phenylphenoxy)-m-chloromethylphenylphosphinic acid,  
p-(m-phenylphenoxy)-m-hydroxyphenylphosphinic acid.

The improvement in lubricity characteristics achieved by the addition of the phenoxyphenylphosphinic acids to the polyphenyl ether base fluid is unusual and surprising. The compositions are particularly useful for steel on steel lubrication.

The compositions of this invention contain a major amount of the polyphenyl ether base stock, i.e., at least 50% by weight of the total composition comprises a polyphenyl ether. It is preferred that at least 60% by weight of the composition be a polyphenyl ether base stock and even more preferred that at least 85% by weight of the total composition comprise a polyphenyl ether.

The compositions of this invention can also contain from 0.01 to 10% by weight of the total composition of a dialkyl hydrogen phosphite extreme pressure additive. The dialkyl hydrogen phosphites useful are those wherein the alkyl groups contain from 1 to 12 carbon atoms. These alkyl groups are, for example, methyl, ethyl, propyl, isopropyl, butyl, sec-butyl, t-butyl, hexyl, decyl isodecyl, dodecyl and the like.

The phenoxyphenylphosphinic acids useful in this invention are prepared by interaction of a phosphine of the formula



wherein R, R<sup>1</sup>, n and a are as defined above with ethyl alcohol and water.

The interaction is carried out in the absence of a solvent by heating the admixture of the three components at temperatures up to and including reflux temperature. Pressure is not critical and subatmospheric, atmospheric and

superatmospheric pressures can be employed. It is generally preferred to slowly add the phosphine to the ethyl alcohol and then to add the water to the admixture of phosphine and ethyl alcohol prior to heating. After reaction is complete, generally a period not exceeding more than ten or fifteen minutes, the excess ethyl alcohol and water are removed by azeotropic distillation with an azeotroping agent such as benzene.

The separation of the desired phosphinic acid from the azeotroping agent is readily accomplished by conventional means well known to the art. For example, distillation, fractional distillation under reduced pressure, selective extraction, fractional distillation using a carrier gas, film distillation, evaporation, elution, or any suitable combination of these methods.

Dichlorophenoxyphenylphosphines can be prepared by Friedel-Craft condensation of diphenyl ethers with phosphorus trichloride in accordance with the procedure set forth in Organic Synthesis, 31, p. 88 (1951).

The following examples serve to further illustrate the invention. All parts are parts by weight unless otherwise expressly set forth.

#### EXAMPLE 1

This example describes the preparation of p-phenoxyphenylphosphinic acid. One part of dichloro-p-phenoxyphenylphosphine (B.P. 138-143° C./0.5 mm, Hg) is slowly added to five parts of absolute ethyl alcohol in a suitable vessel and then two parts of water are added to the alcohol phosphine admixture with continuous stirring. The resulting mixture is heated at reflux for about five minutes. Evaporation of alcohol and water provides an oily substance. Residual alcohol and water are removed from the oily substance by azeotropic distillation using benzene as the azeotroping agent. The benzene is removed from the acid by evaporation producing an oil which slowly crystallizes. The crystals are dried and subjected to recrystallization from benzene and from an admixture of 70% benzene and 30% petroleum ether (B.P. 30-75° C.). The product p-phenoxyphenylphosphinic acid has a melting point of 96.5-98° C. and is confirmed by N.M.R.

#### EXAMPLE 2

A polyphenylether lubricant composition is prepared by combining p-phenoxyphenylphosphinic acid (0.10 gram) with 100 grams of a polyphenyl ether of the following composition:

|                                                  | Percent |
|--------------------------------------------------|---------|
| m-Bis(m-phenoxyphenoxy)benzene                   | 65.0    |
| m-(m-Phenoxyphenoxy)phenyl-p-phenoxyphenyl-ether | 33.0    |
| m-Bis(p-phenoxyphenoxy)benzene                   | 2.0     |

After stirring at 40° C. to dissolve the acid, the mixture is cooled to room temperature and filtered.

The lubrication of the composition is shown with a slow speed four ball machine. A slow speed four ball machine measures the boundary lubricity action of additives. This test is a variation of the well known Shell Four Ball Test in which a ball is rotated against three stationary balls. Wear scars and/or seizure loads measure additive lubricity. In the slow speed instrument the three stationary balls are replaced with circular discs. Standard operating conditions are:

65 3 kg. load  
1 r.p.m.  
Room temperature to 700° F.

The speed of rotation is very low, namely one r.p.m. This equals 0.88 inch/minute. This is done for two reasons. It insures boundary conditions, i.e., metal to metal contact. It also eliminates metal skin temperature flashes which can occur at high speeds. Thus the bulk oil temperature is equivalent to the metal surface temperature. Under these conditions wear is negligible and friction is used to follow lubrication. After covering the ball and

disc with the test oil, the initial friction is recorded. The test sample is then heated at 700° F. with continuous recording of the friction. This gives a boundary friction-temperature profile for the experimental fluid over this temperature range.

The p-phenoxyphenylphosphinic acid/polyphenyl ether composition of this example was tested by this procedure on M-50 tool steel. The base stock was also tested for control purposes. The measured coefficient of friction of the composition of this example was substantially lower than the measured coefficient of friction for the base fluid over the temperature range from 300° F. to 700° F. and particularly from 350° F. to 430° F. and from 500° F. and 700° F.

I claim:

1. Composition comprising a major amount of a polyphenyl ether and from about 0.01 to about 0.5% by weight of a phenoxyphenylphosphinic acid of the formula



wherein R and R<sup>1</sup> are alkyl of not more than 4 carbon atoms, haloalkyl of not more than 4 carbon atoms and 3 halogen atoms, halogen, hydroxyl or phenyl and n and a are integers from 0 to 3.

2. Composition of claim 1 wherein the phenoxyphenylphosphinic acid is present in amounts of from about 0.05 to about 0.2% by weight.

3. Composition of claim 1 wherein the phenoxyphenylphosphinic acid is p-phenoxyphenylphosphinic acid.

4. Composition of claim 1 wherein the phenoxyphenylphosphinic acid is o-phenoxyphenylphosphinic acid.

5. Composition of claim 1 wherein the phenoxyphenylphosphinic acid is m-phenoxyphenylphosphinic acid.

6. Composition of claim 1 wherein R and R<sup>1</sup> are alkyl and n and a are one.

7. Composition of claim 1 wherein R is alkyl, n is one and a is zero.

8. Composition of claim 1 wherein R is phenyl, n is one, and a is zero.

9. Composition of claim 1 wherein R is hydroxyl, n is one and a is zero.

10. Composition of claim 5 wherein R and R<sup>1</sup> are methyl.

#### References Cited

##### UNITED STATES PATENTS

|    |           |         |               |       |            |
|----|-----------|---------|---------------|-------|------------|
| 20 | 2,614,990 | 10/1952 | Harman et al. | ----- | 252—49.9   |
|    | 2,913,415 | 11/1959 | Schmitz       | ----- | 252—49.8 X |

##### FOREIGN PATENTS

|         |         |               |       |          |
|---------|---------|---------------|-------|----------|
| 606,672 | 10/1960 | Canada        | ----- | 252—49.9 |
| 851,651 | 10/1960 | Great Britain | ----- | 252—52 R |

DANIEL E. WYMAN, Primary Examiner

W. H. CANNON, Assistant Examiner

U.S. CL. X.R.

252—49.8, 78; 260—502.4 R